

(No Model.)

P. L. RANDALL.

FIRE KINDLER.

No. 415,734.

Patented Nov. 26, 1889.

Fig. 1.



Fig. 2.



Witnesses:

*E. W. Durman*  
*M. H. Durall*

By his Attorneys,

Parry L. Randall

Inventor

*C. A. Snow & Co.*

# UNITED STATES PATENT OFFICE.

PARRY L. RANDALL, OF PORTSMOUTH, NEW HAMPSHIRE.

## FIRE-KINDLER.

SPECIFICATION forming part of Letters Patent No. 415,734, dated November 26, 1889.

Application filed May 17, 1889. Serial No. 311,115. (No specimens.)

*To all whom it may concern:*

Be it known that I, PARRY L. RANDALL, a citizen of the United States, residing at Portsmouth, in the county of Rockingham and 5 State of New Hampshire, have invented a new and useful Fire-Kindler, of which the following is a specification.

This invention has relation to fire-kindlers, and is intended for kindling the coal direct 10 and without the aid of fire or kindling wood.

Among the objects in view are to provide an inexpensive and safe kindling material formed in convenient blocks adapted to be broken, the nature of the kindler being such 15 as to create when ignited an intense and lasting heat, which, without the aid of kindling-wood, will in a very few moments thoroughly ignite the coal, and this so thoroughly as to render the same capable of creating steam, 20 by which the invention is especially adapted for use in steam-engine boilers, locomotive-boilers, stoves, and, in fact, anywhere wherein it is essential or desirable to provide a quick and intense heat.

25 With these general objects in view the invention consists in the mixing and molding of certain ingredients, and, further, in chemically and otherwise treating the same, all as will hereinafter appear, and be particularly 30 pointed out in the claims.

Referring to the drawings, Figure 1 represents a perspective of a fire-kindler block constructed in accordance with my invention, and Fig. 2 is a transverse section of the same.

35 Like numerals of reference indicate like parts in all the figures of the drawings.

In practicing my invention I first mix thoroughly six parts of finely-sifted wood or coal ashes with one part of calcined plaster and 40 sufficient water to make pliable for molding. By suitable molds, preferably of substantially brick form and having transverse and longitudinal beads or ridges, I form brick-shaped blocks 1, having intersecting channels 2, dividing the block or brick into smaller sections 3. About ten minutes is sufficient to give the block the required form, after which the same is placed in a kiln or oven,

where the water is evaporated and where it is allowed to remain from five to six hours. 50 The block is then removed and permitted to cool, when it will be seen the same is of a very porous nature. I then place this porous block in a tank of unexplosive high-test gas-oil, in which it is allowed to remain some 55 three or four hours, or until thoroughly saturated with the oil. The block is then placed upon suitable brackets or shelves and permitted to drip and partially dry on the outside, after which it is given an outside coating of coal-tar, said tar having been boiled to such a consistence as to harden in a few moments after the coating. The coating of tar seals all the pores of the block and prevents the evaporation of the same and permits the 65 block to be preserved for a great length of time and to retain all its combustible qualities.

By practice I have ascertained that an ordinary hard-coal fire will contain about three 70 gills of oil. After the brick or block has burned out the same will by a slight raking crumble to powder and pass between the grate-bars.

I do not limit my invention to coating the 75 block with coal-tar, as when the block is to be used within a short period of time such preservative is unnecessary.

By practical test I have been able by the employment of this kindler to create thirty 80 pounds of steam in a steam fire-engine in seven minutes and a half.

Having described my invention, what I claim is—

1. A fire-kindler prepared by mixing wood 85 or coal ashes and plaster, molded in any suitable shape, burned or dried, and bathed in oil, as an article of manufacture.

2. A fire-kindler prepared by mixing wood or coal ashes and plaster, molded in any 90 suitable shape, burned or dried, and bathed in oil, and provided with a coating of tar.

3. As a new article of manufacture, a fire-kindler composed of six parts of wood or coal ashes to one part of calcined plaster, 95 mixed together with water, and subsequently

molded and burned to form a porous brick, which is bathed in oil and finally coated with tar, as set forth.

4. The block 1, subdivided into sections 3 and consisting of a mixture of ashes, calcined plaster, and water, molded and dried, bathed in gas-oil, and provided with a coating of coal-tar.

In testimony that I claim the foregoing as my own I have hereto affixed my signature in presence of two witnesses.

PARRY L. RANDALL.

Witnesses:

JOSEPH AUGUSTUS FOUNK,  
S. WESLY HOLLIS.